# EUROPEAN PATENT SPECIFICATION

(11) **EP 2 975 147 B1**
(45) Date of publication and mention of the grant of the patent: **10.01.2018**
(21) Application number: 14762286.4
(22) Date of filing: 12.03.2014
(51) Int. Cl.: C22C 38/00, C22C 38/02, C22C 38/04, C22C 38/06, C22C 38/12, C22C 38/14, C22C 38/60, H01F 1/16, H01F 1/147, C21D 8/12

(54) **NON-ORIENTED ELECTRICAL STEEL SHEET HAVING EXCELLENT HIGH-FREQUENCY IRON LOSS PROPERTY**
NICHTORIENTIERTES ELEKTROSTAHLBLECH MIT AUSGEZEICHNETER HOCHFREQUENZEISENVERLUSTEIGENSCHAFT
FEUILLE D'ACIER ÉLECTRIQUE NON ORIENTÉE AYANT UNE EXCELLENTE PROPRIÉTÉ DE PERTE DE FER À HAUTE FRÉQUENCE

(30) Priority: 15.03.2013 JP 2013053307
(43) Date of publication of application: 20.01.2016
(73) Proprietor: JFE Steel Corporation, Tokyo, 100-0011 (JP)
(72) Inventor: ODA, Yoshihiko, Tokyo 100-0011 (JP); TODA, Hiroaki, Tokyo 100-0011 (JP); KOSEKI, Shinji, Tokyo 100-0011 (JP); HIRATANI, Tatsuhiko, Tokyo 100-0011 (JP); NAKANISHI, Tadashi, Tokyo 100-0011 (JP)
(74) Representative: Stebbing, Timothy Charles
(86) International application number: PCT/JP2014/056426
(87) International publication number: WO 2014/142149

(56) References cited:
- WO-A1-2011/155183
- WO-A1-2011/155183
- CA-A1- 2 821 087
- CN-A- 102 634 742
- JP-A- 2001 335 897
- JP-A- 2001 335 897
- JP-A- 2002 030 397
- JP-A- 2002 047 542
- JP-A- 2002 047 542
- JP-A- 2003 055 746
- JP-A- 2003 055 746
- JP-A- 2003 096 548
- JP-A- 2008 156 737
- JP-A- 2008 156 737
- JP-A- 2008 231 504
- JP-A- 2008 231 504
- JP-A- 2011 179 027
- JP-A- 2012 036 459

## Description

### TECHNICAL FIELD

This invention relates to a non-oriented electrical steel sheet having an excellent high-frequency iron loss property.

### RELATED ART

A motor for hybrid automobiles and electric automobiles is driven at a high-frequency area of 400-2k Hz from a viewpoint of miniaturization and high efficiency. A non-oriented electrical steel sheet used in a core material for such a high-frequency motor is desired to be low in the iron loss at the high frequency.

In order to reduce the iron loss at the high frequency, it is effective to decrease a sheet thickness and increase a specific resistance. However, the method of decreasing the sheet thickness has a problem of lowering the productivity because not only the handling of the material is difficult due to the decrease of its rigidity but also the punching number or stacking number is increased. On the contrary, the method of increasing the specific resistance has not a demerit point as mentioned above, so that it is said to be desirable as a method of decreasing a high-frequency iron loss.

The addition of Si is effective for increasing the specific resistance. However, Si is an element having a large solid-solution strengthening ability, so that there is a problem that the material is hardened with the increase of Si addition amount to deteriorate the rolling property. As a countermeasure for solving this problem, there is a method of adding Mn instead of Si. Since Mn is small in the solid-solution strengthening ability as compared to Si, the high-frequency iron loss can be reduced while suppressing the decrease of the productivity.

For example, as a technique utilizing the above addition effect of Mn, Patent Document 1 discloses a non-oriented electrical steel sheet containing Si: 0.5-2.5 mass%, Mn: 1.0-3.5 mass% and Al: 1.0-3.0 mass%. Also, Patent Document 2 discloses a non-oriented electrical steel sheet containing Si: not more than 3.0 mass%, Mn: 1.0-4.0 mass% and Al: 1.0-3.0 mass%. Patent Document 3 discloses a non-oriented electrical steel sheet containing Si: 1.5-4.0 mass%, Mn: 0.005-2.00 mass% and Sb: 0.005-0.50 mass%. Patent Document 4 discloses a non-oriented electrical steel sheet containing C: 0.005 mass% or less, Si: 1.5-4 mass%, Mn: 1-5 mass%, P: 0.1 mass% or less, S: 0.005 mass% or less, Al: 3 mass% or less and is silent about the presence of Mo. Patent Document 5 discloses a non-oriented electrical steel sheet containing C: 0.002-0.006 mass%, Cr: 0.3-6 mass%, Si: 2-4 mass%, Al: 0.1-3 mass%, Mn: ≤ 1.5%, S: ≤ 0.003 mass%, N: ≤ 0.003 mass% and Mo: 0.005-0.02%. Patent Document 6 discloses a non-oriented electrical steel sheet containing C: ≤ 0.005 mass%, P: ≤ 0.1%, Si: 1.5-5%, Mn: 1-5 mass%, Al: 0.1-3.0 mass%, S: ≤ 0.02 mass% and N: ≤ 0.005 mass%. Patent Document 7 discloses a non-oriented electromagnetic steel sheet containing, in mass%, C: 0.02% or less, Si: 4.5% or less, Mn: 3.0% or less, Al: 3.0% or less and P: 0.50% or less. Patent Document 8 discloses a non-oriented electromagnetic steel sheet containing C: not more than 0.03 mass%, Si: not more than 4 mass%, Mn: 0.03-3 mass%, Al: not more than 3 mass%, S: not more than 0.005 mass% and N: not more than 0.005 mass%. Patent Document 9 discloses a non-oriented silicon steel sheet containing C: ≤ 0.005%, Si: 0.5 to < 3%, Mn: >1.5 to 2.5%, sol.Al: 1-3%, P: ≤ 0.1%, S: ≤ 0.005%, N: ≤ 0.005%, Sn: 0.002-0.2%, Cu: 0.02-0.3%, Ni: 0.01-0.2%, Cr: 0.01-0.2%, V: 0.0005-0.01 %, Nb: 0.001-0.02 % and Ti:≤ 0.01 %. Patent Document 10 discloses a non-oriented magnetic steel sheet containing, by mass, 0.005% or less of C, 1.0-4.0% of Si, 0.1 to 3.0% of sol.Al, 0.1 to 3.0% of Mn, 0.2% or less of P, 0.01% or less of S and 0.01% or less of N. Patent Document 11 discloses a non-oriented silicon steel sheet with a composition containing, by mass, ≤0.005% of C, 0.5 to <3.0% of Si, >1.0 to 3.0% of Mn, 1.0 to 3.0% of sol.Al and ≤0.1 of P.

### PRIOR ART DOCUMENTS

### PATENT DOCUMENTS

- Patent Document 1:: JP-A-2002-047542
- Patent Document 2:: JP-A-2002-030397
- Patent Document 3:: JP-A-2001-335897
Patent Document 4: JP-A-2008-231504Patent Document 5: JP-A-2011-179027Patent Document 6: JP-A-2008-156737Patent Document 7: WO 2011/155183Patent Document 8: CA 2 821 087Patent Document 9: JP-A-2003-096548Patent Document 10: JP-A-2012-036459 Patent Document 11: JP-A-2003-055746

### SUMMARY OF THE INVENTION

### TASK TO BE SOLVED BY THE INVENTION

However, the techniques disclosed in Patent Documents 1 and 2 have a problem that hysteresis loss is increased with the increase of the Mn addition amount and hence the desired effect of reducing the iron loss may not be obtained.

The invention is made in view of the above problem retained in the conventional art and is to provide a non-oriented electrical steel sheet having an excellent high-frequency iron loss property stably even if a great amount of Mn is included.

### SOLUTION FOR TASK

The inventors have made various studies on impurity ingredients included in the steel sheet for solving the above task. As a result, it has been found out that the deterioration of high-frequency iron loss property of a high Mn-added steel is dependent on the presence of Pb included as an impurity and hence high-frequency iron loss can be stably reduced by suppressing a Pb content even in a high Mn content, and the invention has been accomplished.

The invention is based on the above knowledge and is a non-oriented electrical steel sheet having a chemical composition comprising C: not more than 0.005 mass%, Si: 1.5-4 mass%, Mn: 1-5 mass%, P: not more than 0.1 mass%, S: not more than 0.005 mass%, Al: 0.1 3 mass%, N: not more than 0.005 mass%, Pb: not more than 0.0010 mass% and the remainder being Fe and inevitable impurities.

The non-oriented electrical steel sheet according to the invention is characterized by containing one or two of Ca: 0.0005-0.007 mass% and Mg: 0.0002-0.005 mass% in addition to the above chemical composition.

Also, the non-oriented electrical steel sheet according to the invention is characterized by containing one or two of Sb: 0.0005-0.05 mass% and Sn: 0.0005-0.05 mass% in addition to the above chemical composition.

Furthermore, the non-oriented electrical steel sheet according to the invention is characterized by containing Mo: 0.0005-0.0030 mass% in addition to the above chemical composition.

In addition, the non-oriented electrical steel sheet according to the invention is characterized by containing Ti: not more than 0.002 mass%.

### EFFECT OF THE INVENTION

According to the invention, it is possible to stably produce a non-oriented electrical steel sheet having an excellent high-frequency iron loss property by suppressing a content of Pb included as an impurity even if an addition amount of Mn is high.

### BRIEF DESCRIPTION OF THE DRAWINGS

FIG. 1 is a graph showing an influence of Pb content on a relation between Mn content and high-frequency iron loss W_{10/400}.
FIG. 2 is a graph showing a relation between Pb content and high-frequency iron loss W_{10/400}.

### EMBODIEMNTS FOR CARRYING OUT THE INVENTION

An experiment leading to the development of the invention will be first described below.

A steel containing C: 0.0012 mass%, Si: 3.3 mass%, P: 0.01 mass%, S: 0.0005 mass%, Al: 1.3 mass% and N: 0.0021 mass% and added with Mn changing within a range of 0.1-5.5 mass% is melted in a laboratory and shaped into a steel ingot, which is hot rolled, subjected to a hot band annealing at 1000°C in an atmosphere of 100 vol% N₂ for 30 seconds, cold rolled to obtain a cold rolled sheet having a sheet thickness of 0.30 mm and subjected to finishing annealing at 1000°C in an atmosphere of 20 vol% H₂ - 80 vol% N₂ for 30 seconds.

From the thus obtained cold rolled and annealed sheet are cut out specimens for Epstein test with width of 30 mm and length of 280 mm in the rolling direction and a direction perpendicular to the rolling direction and an iron loss W_{10/400} thereof is measured according to JIS C2550.

In FIG. 1, symbol × shows the experimental results as a relation between Mn addition amount and iron loss W_{10/400}. As seen from these results, when Mn content is less than 1 mass%, the iron loss reduces with the increase of Mn addition amount, while the reduction of the iron loss becomes gentle in an amount of not less than 1 mass%, but when it exceeds 4 mass%, the iron loss rather increases. In order to examine this cause, when the steel sheet containing 2 mass% of Mn is observed by TEM, granular Pb compound is found in grain boundaries. As such a steel sheet is further analyzed, Pb is included in an amount of 0.0012-0.0016 mass% as an impurity.

In order to further examine the influence of Pb on the magnetic properties, the iron loss W_{10/400} is measured by melting a steel based on a high-purity steel containing C: 0.0013 mass%, Si: 3.1 mass%, Al: 1.1 mass%, P: 0.01 mass%, S: 0.0005 mass%, N: 0.0025 mass% and Pb: 0.0005 mass% and added with Mn changing within a range of 0.1-5.5 mass% in a laboratory and then shaping into a cold rolled and annealed sheet in the same manner as in the above experiment.

The thus obtained experimental results are shown by symbol ○ in FIG. 1. As seen from these results, the iron loss is reduced in the cold rolled and annealed sheet made from the high-purity steel having a reduced Pb content as the addition amount of Mn is increased as compared to the steel sheet shown by symbol ×. Also, when the steel sheet containing 2 mass% of Mn is observed by TEM, granular Pb compound is not found in grain boundaries. From this result, it is guessed that the increase of the iron loss associated with the increase of Mn addition amount in the steel sheet shown by symbol × is due to the increase of hysteresis loss by precipitation of fine Pb.

In the steel sheet containing Mn of less than 1 mass%, the effect of improving the iron loss by the reduction of Pb is recognized, but the ratio thereof is small, which is not elucidated sufficiently. In the steels having a higher Mn content, it is considered that since the driving force of grain growth is decreased by solute drag of Mn, the grain growth is liable to be largely influenced by the slight amount of Pb.

Pb is generally an impurity incorporated from scraps. Recently, since the use rate of the scraps is increased, not only the amount incorporated but also the dispersion thereof are increased associated therewith. Such an increase of Pb content becomes not a significant problem in the electrical steel sheets having a low Mn content, but the steels having a high Mn content are considered to be largely influenced by the alight amount of Pb since the grain growth is decreased by solute drag of Mn.

In order to examine the influence of Pb content on the iron loss, the iron loss W_{10/400} is measured by melting a steel based on a steel containing C: 0.0020 mass%, Si: 3.15 mass%, Mn: 1.8 mass%, Al: 1.2 mass%, P: 0.01 mass%, S: 0.0006 mass% and N: 0.0017 mass% and added with Pb changing within a range of tr.-0.0060 mass% in a laboratory and then shaping into a cold rolled and annealed sheet of 0.30 mm in thickness in the same manner as in the above experiment.

The experimental results are shown in FIG. 2 as a relation between Pb addition amount and iron loss W_{10/400}. As seen from this figure, the iron loss is highly decreased when the Pb content is not more than 0.0010 mass% (not more than 10 mass ppm). This is considered based on the fact that the grain growth is improved by decreasing the Pb content. From this result, it can be seen that it is necessary to decrease the Pb content to not more than 0.0010 mass% for suppressing the bad influence of Pb on the grain growth. The invention is based on the above novel knowledge.

The chemical composition of the non-oriented electrical steel sheet according to the invention will be described below.

### C: not more than 0.005 mass%

C is an element forming a carbide with Mn. When the content exceeds 0.005 mass%, the amount of Mn-based carbide is increased to obstruct the grain growth, so that the upper limit is 0.005 mass%. Preferably, it is not more than 0.002 mass%.

### Si: 1.5-4 mass%

Si is an element effective for enhancing a specific resistance of steel to reduce the iron loss, so that it is added in an amount of not less than 1.5 mass%. While when it is added in an amount exceeding 4 mass%, the magnetic flux density is decreased, so that the upper limit is 4 mass%. Preferably, the lower limit of Si is 2 mass%, while the upper limit thereof is 3.5 mass%.

### Mn: 1-5 mass%

Mn is an ingredient effective for increasing a specific resistance of steel to reduce the iron loss without largely damaging the workability and is important in the invention, so that it is added in an amount of not less than 1 mass%. In order to more enhance the effect of reducing the iron loss, the addition of not less than 1.6 mass% is preferable. While when it is added in an amount exceeding 5 mass%, the magnetic flux density is decreased, so that the upper limit is 5 mass%. Preferably, the lower limit of Mn is 1.6 mass%, while the upper limit thereof is 3 mass%.

### P: not more than 0.1 mass%

P is an element having a large solid-solution strengthening ability. When it is included in an amount exceeding 0.1 mass%, the steel sheet is significantly hardened to lower the productivity, so that it is restricted to not more than 0.1 mass%. Preferably, it is not more than 0.05 mass%.

### S: not more than 0.005 mass%

S is an inevitable impurity. When it is included in an amount exceeding 0.005 mass%, the grain growth is obstructed by precipitation of MnS to increase the iron loss, so that the upper limit is 0.005 mass%. Preferably, it is not more than 0.001 mass%.

### Al: 0.1-3 mass%

Al is an element effective for enhancing a specific resistance of steel to reduce the iron loss likewise Si. When it is added in an amount exceeding 3 mass%, the magnetic flux density is decreased, so that the upper limit is 3 mass%. Preferably, it is not more than 2 mass%. However, when the Al content is less than 0.1 mass%, fine AlN is precipitated to obstruct the grain growth and increase the iron loss, so that the lower limit is 0.1 mass%.

### N: not more than 0.005 mass%

N is an inevitable impurity penetrated from air into steel. When the content is large, the grain growth is obstructed by precipitation of AlN to increase the iron loss, so that the upper limit is restricted to 0.005 mass%. Preferably, it is not more than 0.003 mass%.

### Pb: not more than 0.0010 mass%

Pb is an important element to be controlled in the invention because it badly affects a high-frequency iron loss property. As seen from FIG. 2, when the Pb content exceeds 0.0010 mass%, the iron loss is violently increased. Therefore, Pb is restricted to not more than 0.0010 mass%. Preferably, it is not more than 0.0005 mass%.

The non-oriented electrical steel sheet according to the invention is preferable to contain one or two of Ca and Mg in addition to the above chemical composition.

### Ca: 0.0005-0.007 mass%

Ca is an element effective for forming a sulfide, precipitating and coarsening together with Pb to suppress harmful action of Pb and reduce the iron loss. In order to obtain such an effect, it is preferable to be added in an amount of not less than 0.0005 mass%. While when it is added in an amount exceeding 0.007 mass%, the amount of CaS precipitated becomes too large and the iron loss is rather increased, so that the upper limit is preferable to be 0.007 mass%. More preferably, the lower limit of Ca is 0.0010 mass%, while the upper limit thereof is 0.0040 mass%.

### Mg: 0.0002-0.005 mass%

Mg is an element effective for forming an oxide, precipitating and coarsening together with Pb to suppress harmful action of Pb and reduce the iron loss. In order to obtain such an effect, it is preferable to be added in an amount of not less than 0.0002 mass%. While when it is added in an amount exceeding 0.005 mass%, the addition itself is difficult and also the increase of the cost is caused unnecessarily, so that the upper limit is preferable to be 0.005 mass%. More preferably, the lower limit of Mg is 0.0005 mass%, while the upper limit thereof is 0.003 mass%.

Moreover, when Ca and/or Mg are added, an acceptable Pb content can be enlarged to 0.0020 mass% by the effect of suppressing the harmful action of Pb.

Furthermore, the non-oriented electrical steel sheet according to the invention is preferable to contain the following ingredients in addition to the above chemical composition.

### Sb: 0.0005-0.05 mass%, Sn: 0.0005-0.05 mass%

Sb and Sn have an effect for improving the texture to increase the magnetic flux density, so that they can be added in an amount of not less than 0.0005 mass% alone or in admixture. More preferably, each of them is not less than 0.01 mass%. However, when each of them is added in an amount exceeding 0.05 mass%, embrittlement of the steel sheet is caused, so that the upper limit of each of them is preferable to be 0.05 mass%.

### Mo: 0.0005-0.0030 mass%

Mo has an effect of coarsening the resulting carbide to reduce the iron loss, so that it is preferable to be added in an amount of not less than 0.0005 mass%. However, when it is added in an amount exceeding 0.0030 mass%, the amount of the carbide becomes too large and hence the iron loss is rather increased, so that the upper limit is preferable to be 0.0030 mass%. More preferably, the lower limit of Mo is 0.0010 mass%, while the upper limit thereof is 0.0020 mass%.

### Ti: not more than 0.002 mass%

Ti is an element forming a carbonitride. When the content is large, the amount of the carbonitride precipitated becomes too large, whereby the grain growth is obstructed to increase the iron loss. In the invention, therefore, Ti is preferable to be limited to not more than 0.002 mass%. More preferably, it is not more than 0.0010 mass%.

Moreover, the remainder other than the aforementioned ingredients in the non-oriented electrical steel sheet according to the invention is Fe and inevitable impurities. However, other elements may be included within a range of not damaging the action and effect of the invention.

Next, there will be described the production method of the non-oriented electrical steel sheet according to the invention.

In the production of the non-oriented electrical steel sheet according to the invention, conditions other than the aforementioned chemical composition of the steel sheet are not particularly limited, so that the steel sheet can be produced under the same conditions as in the usual non-oriented electrical steel sheets as long as the chemical composition is within a range defined in the invention. For example, it can be produced by melting a steel having a chemical composition adapted to the invention in a converter, a degassing device or the like, forming a raw steel material (slab) through continuous casting, ingot making-blooming or the like, hot rolling, hot band annealing as requested, subjecting a single cold rolling or two or more cold rollings sandwiching an intermediate annealing therebetween to a given sheet thickness and subjecting to finishing annealing.

### EXAMPLE

A steel having a chemical composition shown in Table 1 obtained by degassing a molten steel blown in a converter is melted and continuously cast to obtain a slab. The slab is heated at 1100°C for 1 hour, subjected to a hot rolling in which an end temperature of finish rolling is 800°C, wound inform of a coil at a temperature of 610°C to obtain a hot rolled sheet of 1.8 mm in thickness. Then, the hot rolled sheet is subjected to a hot band annealing in an atmosphere of 100 vol% N₂ at 1000°C for 30 seconds, cold rolled to obtain a cold rolled sheet of 0.35 mm in thickness, which is subjected to finishing annealing in an atmosphere of 20 vol% H₂ - 80 vol% N₂ at 1000°C for 10 seconds to obtain a cold rolled and annealed sheet.

From the thus obtained cold rolled and annealed sheet are cut out specimens for Epstein test with a width of 30 mm and a length of 280 mm in the rolling direction and in a direction perpendicular to the rolling direction to measure iron loss W_{10/400} and magnetic flux density B₅₀ according to JIS C2550. The results are also shown in Table 1.

Table 1-1

| No. | Chemical component | | | | | | | (mass%) | | | | | | | Sheet thickness (mm) | Magnetic properties | | Remarks |
|---|---|---|---|---|---|---|---|---|---|---|---|---|---|---|---|---|---|---|
| | C | Si | Mn | P | S | Al | N | Pb | Ca | Mg | Sb | Sn | Mo | Ti | | Iron loss W_{10/400} (W/kg) | Magnetic flux density B₅₀ (T) | |
| 1 | 0.0011 | 3.10 | 1.60 | 0.010 0.0004 | | 1.21 | 0.0012 | 0.0002 | tr. | tr. | tr. | tr. | 0.0010 | 0.0001 | 0.35 | 15.10 | 1.67 | Invention steel |
| 2 | 0.0014 | 3.10 | 1.60 | 0.012 | 0.0004 | 1.21 | 0.0016 | 0.0005 | tr. | tr. | tr. | tr. | 0.0010 | 0.0001 | 0.35 | 15.15 | 1.67 | Invention steel |
| 3 | 0.0021 | 3.12 | 1.60 | 0.011 | 0.0004 | 1.21 | 0.0015 | 0.0005 | tr. | tr. | tr. | tr. | 0.0010 | 0.0001 | 0.35 | 15.30 | 1.67 | Invention steel |
| 4 | 0.0016 | 3.11 | 1.60 | 0.012 | 0.0004 | 1.21 | 0.0017 | 0.0015 | tr. | tr. | tr. | tr. | 0.0010 | 0.0002 | 0.35 | 15.61 | 1.67 | Comparative steel |
| 5 | 0.0011 | 3.10 | 1.60 | 0.012 | 0.0004 | 1.21 | 0.0018 | 0.0025 | tr. | tr. | tr. | tr. | 0.0010 | 0.0002 | 0.35 | 16.11 | 1.67 | Comparative steel |
| 6 | 0.0013 | 3.12 | 0.50 | 0.012 | 0.0004 | 1.21 | 0.0020 | 0.0002 | tr. | tr. | tr. | tr. | 0.0010 | 0.0002 | 0.35 | 16.00 | 1.69 | Comparative steel |
| 7 | 0.0015 | 3.12 | 1.30 | 0.012 | 0.0004 | 1.21 | 0.0020 | 0.0002 | tr. | tr. | tr. | tr. | 0.0010 | 0.0002 | 0.35 | 15.41 | 1.68 | Invention steel |
| 8 | 0.0014 | 3.13 | 1.60 | 0.012 | 0.0004 | 1.21 | 0.0021 | 0.0002 | tr. | tr. | tr. | tr. | 0.0010 | 0.0002 | 0.35 | 15.26 | 1.68 | Invention steel |
| 9 | 0.0013 | 3.09 | 2.50 | 0.012 | 0.0004 | 1.21 | 0.0018 | 0.0002 | tr. | tr. | tr. | tr. | 0.0010 | 0.0002 | 0.35 | 15.06 | 1.66 | Invention steel |
| 10 | 0.0012 | 3.11 | 3.50 | 0.012 | 0.0004 | 1.21 | 0.0016 | 0.0002 | tr. | tr. | tr. | tr. | 0.0010 | 0.0002 | 0.35 | 14.92 | 1.65 | Invention steel |
| 11 | 0.0016 | 3.10 | 5.50 | 0.010 | 0.0004 | 1.00 | 0.0022 | 0.0002 | tr. | tr. | tr. | tr. | 0.0010 | 0.0002 | 0.35 | 15.55 | 1.60 | Comparative steel |
| 12 | 0.0013 | 3.11 | 0.50 | 0.012 | 0.0004 | 1.21 | 0.0015 | 0.0025 | tr. | tr. | tr. | tr. | 0.0010 | 0.0002 | 0.35 | 16.12 | 1.67 | Comparative steel |
| 13 | 0.0016 | 3.12 | 1.55 | 0.012 | 0.0004 | 1.21 | 0.0017 | 0.0005 | tr. | tr. | tr. | tr. | 0.0010 | 0.0002 | 0.35 | 15.25 | 1.67 | Invention steel |
| 14 | 0.0018 | 3.12 | 1.56 | 0.012 | 0.0004 | 1.21 | 0.0020 | 0.0005 | tr. | tr. | 0.0050 | tr. | 0.0010 | 0.0002 | 0.35 | 15.16 | 1.68 | Invention steel |
| 15 | 0.0020 | 3.13 | 1.56 | 0.012 | 0.0004 | 1.21 | 0.0017 | 0.0005 | tr. | tr. | 0.0180 | tr. | 0.0010 | 0.0002 | 0.35 | 15.15 | 1.69 | Invention steel |
| 16 | 0.0020 | 3.12 | 1.56 | 0.012 | 0.0004 | 1.21 | 0.0018 | 0.0005 | tr. | tr. | tr. | 0.0080 | 0.0010 | 0.0002 | 0.35 | 15.15 | 1.68 | Invention steel |
| 17 | 0.0021 | 3.12 | 1.56 | 0.012 | 0.0004 | 1.21 | 0.0020 | 0.0005 | tr. | tr. | tr. | 0.0120 | 0.0010 | 0.0002 | 0.35 | 15.10 | 1.69 | Invention steel |
| 18 | 0.0018 | 3.12 | 1.57 | 0.012 | 0.0004 | 1.21 | 0.0019 | 0.0005 | tr. | tr. | tr. | 0.0350 | 0.0010 | 0.0002 | 0.35 | 15.02 | 1.69 | Invention steel |
| 19 | 0.0016 | 3.12 | 1.58 | 0.012 | 0.0004 | 1.21 | 0.0019 | 0.0005 | 0.0020 | tr. | tr. | tr. | 0.0010 | 0.0002 | 0.35 | 14.91 | 1.67 | Invention steel |

**Table 1-2**

| No. | Chemical component (mass%) | | | | | | | | | | | | | | Sheet thickness (mm) | Magnetic properties | | Remarks |
|---|---|---|---|---|---|---|---|---|---|---|---|---|---|---|---|---|---|---|
| | C | Si | Mn | P | S | Al | N | Pb | Ca | Mg | Sb | Sn | Mo | Ti | | Iron loss (W/kg) | Magnetic flux densityB₅₀ (T) | |
| 22 | 0.0015 | 3.11 | 1.59 | 0.012 | 0.0004 | 1.21 | 0.0021 | 0.0016 | 0.0090 | tr. | tr. | tr. | 0.0010 | 0.0002 | 0.35 | 15.56 | 1.67 | Comparative steel |
| 23 | 0.0016 | 3.12 | 1.61 | 0.012 | 0.0004 | 1.21 | 0.0018 | 0.0030 | 0.0030 | tr. | tr. | tr. | 0.0010 | 0.0002 | 0.35 | 15.63 | 1.67 | Comparative steel |
| 24 | 0.0015 | 3.12 | 1.61 | 0.012 | 0.0004 | 1.21 | 0.0016 | 0.0005 | tr. | 0.0010 | tr. | tr. | 0.0010 | 0.0002 | 0.35 | 14.92 | 1.67 | Invention steel |
| 27 | 0.0021 | 1.00 | 1.62 | 0.030 | 0.0004 | 2.50 | 0.0017 | 0.0005 | tr. | tr. | tr. | tr. | 0.0010 | 0.0002 | 0.35 | 18.50 | 1.67 | Comparative steel |
| 29 | 0.0014 | 3.13 | 1.60 | 0.012 | 0.0004 | 1.21 | 0.0021 | 0.0002 | tr. | tr. | tr. | tr. | 0.0020 | 0.0002 | 0.35 | 15.26 | 1.68 | Invention steel |
| 30 | 0.0014 | 3.13 | 1.60 | 0.012 | 0.0004 | 1.21 | 0.0021 | 0.0002 | tr. | tr. | tr. | tr. | 0.0029 | 0.0002 | 0.35 | 15.41 | 1.68 | Invention steel |
| 31 | 0.0020 | 2.20 | 1.30 | 0.012 | 0.0004 | 2.00 | 0.0020 | 0.0005 | tr. | tr. | tr. | tr. | 0.0010 | 0.0002 | 0.35 | 15.10 | 1.67 | Invention steel |
| 32 | 0.0016 | 3.50 | 1.10 | 0.005 | 0.0004 | 1.00 | 0.0017 | 0.0005 | tr. | tr. | tr. | tr. | 0.0010 | 0.0002 | 0.35 | 14.82 | 1.67 | Invention steel |
| 33 | 0.0015 | 4.70 | 1.10 | 0.005 | 0.0004 | 0.30 | 0.0018 | 0.0005 | tr. | tr. | tr. | tr. | 0.0010 | 0.0002 | 0.35 | 14.51 | 1.60 | Comparative steel |
| 34 | 0.0015 | 2.80 | 1.60 | 0.012 | 0.0004 | 1.30 | 0.0015 | 0.0005 | tr. | tr. | tr. | tr. | 0.0010 | 0.0002 | 0.35 | 14.97 | 1.67 | Invention steel |
| 35 | 0.0017 | 2.50 | 1.60 | 0.012 | 0.0004 | 2.50 | 0.0016 | 0.0005 | tr. | tr. | tr. | tr. | 0.0010 | 0.0002 | 0.35 | 14.72 | 1.67 | Invention steel |
| 36 | 0.0019 | 1.50 | 1.60 | 0.012 | 0.0004 | 3.50 | 0.0018 | 0.0005 | tr. | tr. | tr. | tr. | 0.0010 | 0.0002 | 0.35 | 14.98 | 1.62 | Comparative steel |
| 37 | 0.0017 | 2.80 | 1.60 | 0.012 | 0.0015 | 1.30 | 0.0016 | 0.0005 | tr. | tr. | tr. | tr. | 0.0010 | 0.0002 | 0.35 | 15.20 | 1.65 | Invention steel |
| 38 | 0.0018 | 2.80 | 1.60 | 0.012 | 0.0060 | 1.30 | 0.0014 | 0.0005 | tr. | tr. | tr. | tr. | 0.0010 | 0.0002 | 0.35 | 17.30 | 1.65 | Comparative steel |
| 39 | 0.0015 | 2.80 | 1.60 | 0.012 | 0.0005 | 1.30 | 0.0016 | 0.0005 | tr. | tr. | tr. | tr. | 0.0010 | 0.0035 | 0.35 | 16.30 | 1.66 | Comparative steel |
| 40 | 0.0015 | 2.80 | 1.60 | 0.012 | 0.0004 | 1.30 | 0.0065 | 0.0005 | tr. | tr. | tr. | tr. | 0.0010 | 0.0002 | 0.35 | 16.60 | 1.65 | Comparative steel |
| 41 | 0.0069 | 2.80 | 1.60 | 0.012 | 0.0004 | 1.30 | 0.0013 | 0.0005 | tr. | tr. | tr. | tr. | 0.0010 | 0.0002 | 0.35 | 16.40 | 1.66 | Comparative steel |

As seen from Table 1, the steel sheets satisfying the chemical composition defined in the invention, particularly steel sheets having a reduced Pb content are excellent in the high-frequency iron loss property irrespectively of a high Mn content.

### INDUSTRIAL APPLICABILITY

The invention can also be applied to a motor for working machine, a motor for hybrid EV, a high-speed generator and so on.

## Claims

1. A non-oriented electrical steel sheet having a chemical composition consisting of C: not more than 0.005 mass%, Si: 1.5-4 mass%, Mn: 1-5 mass%, P: not more than 0.1 mass%, S: not more than 0.005 mass%, Al: 0.1-3 mass%, N: not more than 0.005 mass%, Pb: not more than 0.0010 mass%, Mo: 0.0005-0.0030 mass%, Ti: not more than 0.002 mass%, optionally one or two of Ca: 0.0005-0.007 mass% and Mg: 0.0002-0.005 mass%, optionally one or two of Sb: 0.0005-0.05 mass% and Sn: 0.0005-0.05 mass%, and the remainder being Fe and inevitable impurities.

## Patentansprüche

1. Nichtorientiertes Elektrostahlblech, das eine chemische Zusammensetzung aufweist, die aus Folgenden besteht: C: nicht mehr als 0,005 Masse-%, Si: 1,5 -4 Masse-%, Mn: 1 - 5 Masse-%, P: nicht mehr als 0,1 Masse-%, S: nicht mehr als 0,005 Masse-%, Al: 0,1 - 3 Masse-%, N: nicht mehr als 0,005 Masse-%, Pb: nicht mehr als 0,0010 Masse-%, Mo: 0,0005 - 0,0030 Masse-%, Ti: nicht mehr als 0,002 Masse-%, wahlweise einem oder zwei von Ca: 0,0005 - 0,007 Masse-% und Mg: 0,0002 - 0,005 Masse %, wahlweise einem oder zwei von Sb: 0,0005 - 0,5 Masse-% und Sn: 0,0005 - 0,05 Masse-%, und wobei der Rest Fe und unvermeidliche Verunreinigungen ist.

## Revendications

1. Tôle d'acier électrique non orientée ayant une composition chimique composée de C : pas plus de 0,005 % en masse, Si : 1,5-4 % en masse, Mn : 1-5 % en masse, P : pas plus de 0,1 % en masse, S : pas plus de 0,005 % en masse, Al : 0,1-3 % en masse, N : pas plus de 0,005 % en masse, Pb : pas plus de 0,0010 % en masse, Mo : 0,0005-0,0030 % en masse, Ti : pas plus de 0,002 % en masse, de manière facultative un ou deux parmi Ca : 0,0005-0,007 % en masse et Mg : 0,0002-0,005 % en masse, de manière facultative un ou deux parmi Sb : 0,0005-0,05 % en masse et Sn : 0,0005-0,05 % en masse, et le reste étant Fe et des impuretés inévitables.
